

Patented May 8, 1928.

1,668,934

# UNITED STATES PATENT OFFICE.

RUSSELL S. BRACEWELL, OF SOUTH HADLEY, MASSACHUSETTS, ASSIGNOR TO THE MARVELLUM COMPANY, A CORPORATION OF MASSACHUSETTS.

## PROCESS OF DYE PRINTING FABRICS WITH A FREE NONREPEAT DESIGN.

No Drawing.

Application filed May 18, 1925. Serial No. 31,216.

The present invention relates to a process of ornamenting textile fabrics and more particularly to a method of dyeing such fabrics with a free non-repeat pattern or variegated design.

The usual method of printing designs on fabrics by engraved rollers and the like does not lend itself to a continuous variation in detail of the design without prohibitive expense whereas in the present improved process a continuous application of the design may be made differing more or less in detail at the will of the operator and yet having a general appearance of sameness or uniformity. Such designs known as a marbling effect have heretofore been applied to paper as a coating thereon, but a fabric similarly coated, necessarily with pigment or lake colors carried in some oxidizable oil as a vehicle, is open to the same objections as a painted fabric. The natural lustre of the fabric is thereby covered up and destroyed and the stiffness of the oxidized oil and pigment on the surface gives the fabric a harsh feel and prevents proper draping.

The foregoing objections are avoided in the present process which contemplates the actual dyeing of the fabric with the design and in a manner to fix the color into the pores of the fiber so as to be fast to light and washing. All extraneous agents are removed at the completion of the process so that the finished fabric will have the same feel and quality as any other dyed fabric of similar nature. For this purpose, I employ insoluble dyes known as vat dyes and of similar nature in this respect to indigo. Insoluble sulphur dyes may likewise be used. The dye or dyes in their insoluble form are applied to the fabric in the manner herein-after described, are reduced to their soluble state while on the fabric for penetrating thoroughly into the fibers and are finally set on the fiber by oxidization which restores them to their insoluble condition and gives the fabric its permanently dyed character.

In amplification of the foregoing general statements, the present invention will now be more particularly described. It will be understood of course that the character of the design desired will determine the use of one dye or several dyes of different color, but all having the same character of insolubility described above, which may be jointly employed in the present process. In

the following description, therefore, it is necessary to consider the action of only one dye color.

The insoluble dye is ground to a very fine state of division in a fixed oil of the character of olive oil. Other suitable vegetable slow-drying oils which do not oxidize too readily may be used, but so far I have found olive oil best suited to the purpose. The pasty ground mixture of dye and olive oil should be thinned down to an easy flowing state by the addition of more fixed oil and of a lighter oil such as benzol or other similar volatile oil. It is desirable to add a filler such as stearine or other similar filler to the mixture to bring about proper working qualities of the color mixture. For the mixture thus obtained, which may be termed the color mixture, the oils are so chosen as to obtain good penetration of the color into the fabric and as the oils are to be subsequently removed they must be capable of being volatilized or saponified and emulsified. The filler along with the oil both before and after saponification serves to hold the color in the design field of the fabric and prevents running.

The color mixture when prepared is then distributed upon the surface of a liquid carrier which should be a non-solvent for the mixture. Such a liquid carrier may be water or a suitable water solution commonly used for the same purpose in the process of marbling paper. The color mixture forms a floating film of mutable design upon the surface of the water and may be swirled about by any of the known methods to obtain the free non-repeat pattern or variegated design desired for transfer to the fabric.

The fabric is then brought into surface contact with the liquid carrier to take up the floating film of color design therefrom, and any of the well known methods, either by hand or by machine, may be employed for this purpose. For the commercial production of designs on long webs or rolls of cloth some suitable apparatus would be necessary and such an apparatus is described in a copending application filed December 29, 1924, Serial No. 758,632, of which I am a joint inventor.

After the transfer of the film of color mixture to the cloth, the water taken up with the film and the volatile oils in the mixture

are driven off by a drying heat. The cloth carrying the dye still in its insoluble form and merely held in the oil is then subjected to the action of a reducing agent to reduce 5 the dye to its soluble form for penetration into the fibers of the cloth. This may be accomplished in several ways, two of which will be described.

According to one method, the cloth may 10 be immersed in a bath of alkaline hydrosulphite, for instance sodium hydrosulphite in the presence of sufficient lime or soda. The time of immersion and the temperature of the bath will depend on the nature of the 15 dye being used and the strength of the alkali will be varied to suit the particular fabric in question.

According to another method, and which in some respects is perhaps preferable to the 20 first described, the rear side of the fabric, i. e., opposite to that on which the film of color mixture has been applied, is run in contact with a transfer roll which delivers to and presses into the rear side of the fabric a 25 thickened solution of the alkaline hydrosulphite. Instead of employing such a transfer roll, the rear side of the fabric may be drawn over a slotted pipe through which a thickened solution of the alkaline hydrosulphite 30 may be forced under pressure into the fabric. In either case, the alkaline hydrosulphite is mixed with a suitable size, such as gum, glue or starch to give it body and prevent the dye running in the fabric.

35 When the alkaline hydrosulphite is applied to the rear side of the fabric by rolls or pressure pipes as described, it is thereafter baked or cooked in the fabric to increase its effectiveness in reducing the insoluble dye. 40 This cooking may be accomplished by carrying the fabric over hot drums or through an oven. After being thus heated or cooked, the fabric should stand a while for aging, twenty-four hours preferably, which completes the reduction of the dye and allows it 45 to thoroughly penetrate in to the pores of the fiber.

The effect of the alkaline reducing agent, either when applied in the bath or by the 50 direct method of pressure is both to saponify the non-volatile oil of the mixture and render the dye soluble for penetration into the fiber. The dye is then ready for being set or fixed in the fiber and the oil is in condition 55 for subsequent removal. The next step is to wash the fabric in cold water when the start of the oxidization action on the reduced dye may be noted and at this stage the fabric may or may not be aged in a box of 60 live steam to further oxidize and fix the dye.

For the final oxidization of certain dyes and permanent fixing of the same in the fiber, the fabric is then immersed in an acid bath of dichromate, such for instance as a 65 solution of potassium dichromate in acetic

acid, which renders the dye again insoluble and in condition to firmly adhere to the fibers in the manner of such dyes. For other dyes which oxidize more easily this change is effected by merely exposing to the air.

70 After the final fixing of the dye, the fabric is then washed in a bath of water to remove the excess acid and dichromate and finally washed in a soap bath of boiling water to remove the saponified oil filler and other extraneous substances leaving the fabric ready to be finished in the usual way of finishing textiles. This boiling in soap bath for most dyes brings out the tone and makes them 80 faster. The dyed fabric will then show its final shade.

85 The invention as hereinafter claimed should not be limited to the details of the process above described since obviously different but equivalent steps to those pointed out may be adopted and other equivalent substances having the same effect as those specifically mentioned may be equally well employed to accomplish like results.

90 What I claim is:

1. The process of dyeing fabrics with a variegated non-repeat design which consists in forming an easy flowing color mixture of a finely divided insoluble dye with an oil, distributing said color mixture upon the surface of a non-solvent liquid carrier to form a floating film of mutable design, bringing the fabric into surface contact with said liquid carrier to take up the floating film therefrom, subjecting the color mixture thus on the fabric to the action of a reducing agent for rendering said dye soluble for penetration into said fabric, and then oxidizing said reduced soluble dye to its insoluble state for fixing the same in the fabric.

95 2. The process of dyeing fabrics with a variegated non-repeat design which consists in forming an easy flowing color mixture of a finely divided insoluble dye with an oil capable of saponification, distributing said color mixture upon the surface of a non-solvent liquid carrier to form a floating film of mutable design, bringing the fabric into surface contact with said liquid carrier to take up the floating film therefrom, subjecting the color mixture thus on the fabric to the action of an alkaline reducing agent for rendering said dye soluble for penetration into said fabric and for saponifying said oil to facilitate removal thereof, and then oxidizing said reduced soluble dye to its insoluble state for fixing the same in the fabric.

100 3. The process of dyeing fabrics with a variegated non-repeat design which consists in forming an easy flowing color mixture of a finely divided insoluble dye with a slow 105 drying fixed oil capable of saponification, distributing said color mixture upon the surface of a non-solvent liquid carrier to

- form a floating film of mutable design, bringing the fabric into surface contact with said liquid carrier to take up the floating film therefrom, subjecting the color mixture 5 thus on the fabric to the action of an alkaline reducing agent for rendering said dye soluble for penetration into said fabric and for saponifying said oil to facilitate removal therefrom, and then oxidizing said reduced 10 soluble dye to its insoluble state for fixing the same in the fabric.
4. The process of dyeing fabrics with a variegated non-repeat design which consists in forming an easy flowing color mixture of 15 a finely divided insoluble dye with a slow drying fixed oil capable of saponification and suitably thinned with a lighter volatile oil, distributing said color mixture upon the surface of a non-solvent liquid carrier to form 20 a floating film of mutable design, bringing the fabric into surface contact with said liquid carrier to take up the floating film therefrom, subjecting the color mixture thus on the fabric to the action of an alkaline 25 reducing agent for rendering said dye soluble for penetration into said fabric and for saponifying said oil to facilitate removal thereof, and then oxidizing said reduced 30 soluble dye to its insoluble state for fixing the same in the fabric.
5. The process of dyeing fabrics with a variegated non-repeat design which consists in forming an easy flowing color mixture of a finely divided insoluble dye with a 35 slow drying fixed oil capable of saponification and suitably thinned with a lighter volatile oil, said mixture containing a filler to prevent running of the color in the fabric, distributing said color mixture upon the 40 surface of a non-solvent liquid carrier to form a floating film of mutable design, bringing the fabric into surface contact with said liquid carrier to take up the floating film therefrom, subjecting the color mixture 45 thus on the fabric to the action of an alkaline reducing agent for rendering said dye soluble for penetration into said fabric and for saponifying said oil to facilitate removal thereof, and then oxidizing said reduced 50 soluble dye to its insoluble state for fixing the same in the fabric.
6. The process of dyeing fabrics with a variegated non-repeat design which consists in forming an easy flowing color mixture of a finely divided insoluble dye with a slow drying fixed oil capable of saponification and suitably thinned with a lighter volatile oil, distributing said color mixture upon the surface of a non-solvent liquid such as water or a water solution, to form a 60 floating film of mutable design, bringing the fabric into surface contact with said liquid carrier to take up the floating film therefrom, driving off by a drying heat the volatile oil and water taken up by said fabric, subjecting the color mixture on the fabric to the action of an alkaline reducing agent accompanied by heat for rendering said dye soluble and for saponifying said fixed oil, subjecting said dyed fabric to the action of a 65 liquid oxidizing agent to fix the dye in the fabric, and finally washing the fabric in a soap bath for removing the saponified oil and excess of other agents.
7. The process of dyeing fabrics with a variegated non-repeat design which consists in forming an easy flowing color mixture of a finely divided insoluble dye with a slow drying fixed oil, similar to olive oil, capable of saponification and suitably thinned with a lighter volatile oil, distributing said color mixture upon the surface of a non-solvent liquid, similar to water or a water solution, to form a floating film of mutable design, bringing the fabric into 80 surface contact with said liquid carrier to take up the floating film therefrom, driving off by a drying heat the volatile oil and water taken up by said fabric, subjecting the color mixture on the fabric to the action of an alkaline reducing agent similar to an alkaline solution of hydrosulphite accompanied by heat for rendering said dye soluble and for saponifying said fixed oil, subjecting said dye fabric to the action of a 85 liquid oxidizing agent similar to an acid solution of a dichromate to fix the dye in the fabric, and finally washing the fabric in a soap bath for removing the saponified oil and excess of other agents.

In testimony whereof I have affixed by signature.

RUSSELL S. BRACEWELL. [L. S.]